

## UNITED STATES PATENT OFFICE

MELDRUM D. SHANNON, OF SACRAMENTO, CALIFORNIA

## METHOD OF PREPARING PAVEMENT COMPOSITION

No Drawing.

Application filed June 16, 1925. Serial No. 37,581.

The invention relates to a method of preparing a bituminous pavement composition and has for its objects to provide a pavement composition which is extremely durable under continued usage, economical of manufacture and which adheres with a maximum tenacity to different characters of bases or foundations on which it is laid.

A further object of the invention is to provide a road of pavement composition which may be applied with equal facility to a base of concrete, cement, or wood flooring or pavement, without the necessity of interposing a coating of adhesive material, and this is made possible by reason of the nature and mode of preparation of the improved composition.

A further object of the invention is to provide a pavement composition of high wear-resisting qualities and which may be used to equal advantage for either outdoor or indoor purposes.

A further object of the invention is to provide a pavement or flooring composition of the character described, the long durability and high wear-resisting qualities of which are largely due to the increased temperature at which the materials are combined and mixed, and which high temperature it has been found disadvantageous to employ in past and present road and floor building practice.

A further object of the invention is to provide a paving and flooring material which is elastic and which is capable of contracting and expanding without altering or impairing its desirable qualities.

A further object of the invention is to provide a paving material which is fire-proof, acid-proof, and a non-conductor of electricity, with the result that it is especially adaptable for a wear-resisting composition suitable to be laid as a flooring surface in factories, warehouses, and the like.

It has been found in prior practice of laying bituminous pavements and flooring surfaces of the general character contemplated by the present invention, that engineers and contractors have agreed that the asphalt should not be heated to over three

hundred and fifty (350) degrees Fahr. This is for the reason that it is contended that its qualities would thereby be seriously impaired, as well as incurring the possibility of serious explosions. The heating temperature beyond this point has resulted in burning the asphalt; consequently its elasticity is destroyed, its viscosity impaired and the volatile oils eliminated or materially reduced.

In preparing and laying the composition contemplated by the present invention, the best results are obtained by heating the composition, including the asphalt and other combined ingredients as a mixture, to at least three hundred and eighty (380) degrees Fahr. and more advantageous results are obtained when it is heated as high as four hundred and twenty-five (425) degrees Fahr.

This relatively higher temperature obtained by the present invention, and which has heretofore been deemed impracticable, is not attended by any of the disadvantages above set forth and heretofore experienced, and due to the increased temperature herein obtained the material is more intimately mixed and adheres more firmly to the wood or concrete base on which it is laid.

It is extremely difficult to remove because it tends to adhere firmly to the wood fiber or cement, and this extremely high tenacity of the pavement composition toward the base is effected by heating the material to the relatively higher temperatures above outlined, such temperatures of preference not exceeding four hundred and twenty-five (425) degrees Fahr. No intervening coating of paint or other material is

necessary to effect the union between the pavement and the board or base, as has been necessary in other forms of asphalt or bituminous pavement.

With such objects in view, as well as other advantages which may be incident to the use of my improvements, the invention consists in the combination of ingredients and manner of making the same, which are hereinafter set forth and claimed, with the understanding that the several necessary elements and steps of procedure which constitute the same may be varied in proportions

55

60

65

70

75

80

85

90

95

100

without departing from the nature and scope of the invention.

The improved pavement composition which provides the road or flooring surface having the qualities and advantages above set forth, is preferably composed of the following raw ingredients of the nature and character described and which are proportioned and combined in the manner herein-after specified.

*Asphaltic cement.*—The asphaltic cement consists preferably of any standard asphalt, free from admixture with any residues obtained by the artificial distillation of coal, 5 coal tar, or paraffine oil. It is preferably soluble in carbon disulphide to the extent of at least 99 percent, and in carbon tetrachloride to the extent of not less than 98 percent. The asphaltic cement preferably 15 should have a penetration of not more than forty-five degrees, District of Columbia standard.

*Limestone.*—The mineral filler preferably consists of a limestone powdered or pulverized to such degree of fineness that it will entirely pass through a fifty mesh to the 20 inch screen and a minimum of sixty-six percent should pass through a two hundred mesh to the inch screen.

*Sand.*—The sand consists preferably of the clean, hard grained and moderately sharp grade, and should contain not more than three percent of mica, loam, clay, or other earthy impurities. It should of preference contain not less than three percent of 35 moisture.

*Rock.*—The broken stone ingredient preferably consists of clean, hard, and tough rock which should be free from disintegrating 40 material. It is desirable that all of the broken or crushed rock should pass through a three-eighths inch mesh screen.

An enduring wear-resisting pavement or flooring surface consisting of the above ingredients and possessing other desirable attributes above set forth, is preferably or may be prepared by combining and mixing the respective ingredients by weight within 45 the following proportions:

50 (1) Asphaltic cement between 8 and 20 percent.

(2) Finely pulverized stone dust or powdered limestone between 11 and 25 percent.

(3) Sand between 18 and 55 percent.

55 (4) Crushed rock between 14 and 45 percent.

The paving composition may be prepared directly in the vicinity of the road, pavement or flooring to be laid, and the procedure consists in combining and mixing the above ingredients within the proportions specified, in 60 a rotary drum. The drum is provided with an opening to admit air and to permit steam and gases to escape, and is preferably set 65 in a suitable fire box. It is desirable for best

results that the cooking and mixing of the composition be continued at a relatively high temperature until all steam has been driven off the product, the rotation of the drum co-operating with the high degree of temperature to produce a homogeneous, intimately combined flowing product which may be delivered from the mixing drum directly on the surface to be paved. For effective results the temperature at which the composition is delivered from the drum is substantially between three hundred and seventy-five (375) and four hundred and twenty-five (425) degrees Fahr., and it is desirable that the material be delivered from the drum without coming in contact with the flue gases from the fire box.

The composition is laid on or applied to the surface or flooring to be paved while the latter is clean and dry, and effective results are obtained by laying the paving composition in a uniform thickness of approximately three-fourths of an inch. The thickness of the paved surface, however, may be varied according to prevailing conditions. If desired, the mixture may be conveyed from the drum to the surface to be paved in a suitable cart or dump truck, it being desirable that the temperature of said mixture be not lower than three hundred and twenty-five (325) degrees Fahr. at the time it is applied to the surface or base.

In constructing the road, pavement or flooring surface, the composition is prepared as above outlined, is then uniformly spread over the foundation by means of suitable rakes or implements, and is preferably finished to a true and level surface by means of a straight edge. If desired, the material may be of such consistency that it will float into position and after hardening, a suitable roller may be used for smoothing. A small amount of powdered limestone or cement may be thereafter dusted over the surface. The resulting pavement produces a close grained, level, smooth surface of a durable, high wear-resisting quality, possesses a high degree of tenacity or capacity to adhere to the base or foundation, and is free from all depressions and inequalities.

If desired, the improved paving or flooring composition may be prepared by means of a rotary drum heated to the above described relatively high temperature and utilizing most of the ingredients in the proportions specified, but omitting the broken rock. It has been found in practice that an enduring and otherwise satisfactory pavement or flooring may be obtained by the use of asphaltic cement, powdered limestone, and sand alone, 110 when prepared in the manner and proportions above set forth.

It will be understood that the improved and enduring wearing surface, which is provided by preparing the ingredients accord-

ing to the procedure outlined, is largely effected by reason of the relatively high temperature of between three hundred and seventy-five (375) and four hundred and twenty-five (425) degrees Fahr. to which the materials are subjected when intimately combined. This increased and relatively higher temperature over prior practice produces a paving surface which is extremely adherent to the base or foundation on which it is laid. It is especially adherent, by reason of its method of preparation and application, to a base of wood or fiber, thereby rendering the paving composition especially adaptable for covering wooden bridges, factory floorings and the like. In obtaining the above described results, an asphaltic cement below forty-five (45) degrees penetration is preferably employed in the composition.

Satisfactory results have been obtained without the necessity of rolling, tamping, or otherwise compressing the pavement after it has been laid, and this is due to the thorough and intimate mixture of the ingredients at the relatively high temperature described. In the event that it is desired to use a roller for smoothing the finished pavement, a small hand roller weighing not over 500 pounds is sufficient to finally finish the surface.

While the improved composition has been described as particularly applicable for road and pavement surfaces, it is to be understood that the same may be applied with equal satisfactory results as a roofing composition. The material is particularly useful on flat roofs where a waterproof, fire-resisting and long wearing surface is essential and desired. In addition to the useful advantages above set forth, the improved composition is proof against acids, vermin, and does not corrode or crumble away under continued and heavy usage when employed as a building or factory flooring.

What I claim is:

1. The method of preparing a pavement composition which consists in combining a mixture of asphalt, powdered limestone, and sand containing not less than 3 percent of moisture, said materials being thereafter subjected to a temperature in excess of 375 degrees Fahr.

2. The method of producing a pavement and flooring composition which comprises preparing and combining a mixture of asphaltic cement, powdered limestone, broken rock and sand containing substantially three percent or more of moisture, said materials being intimately combined by subjecting the same to a temperature of substantially 375 degrees Fahr. and until practically all steam has been driven off the product.

3. The method of preparing a pavement composition which consists in combining be-

tween 8 and 20 per cent by weight of asphalt, between 11 and 25 percent by weight of powdered limestone, between 18 and 55 percent by weight of sand containing not less than 3 percent of moisture, and between 14 and 45 percent by weight of crushed rock, said materials being intimately combined and heated at a temperature in excess of 375 degrees Fahr., until all steam has been driven off and whereby said composition is made adhesive.

In testimony whereof I affix my signature.  
MELDRUM D. SHANNON.

80

85

90

95

100

105

110

115

120

125

130